

Sept. 10, 1929.

R. E. COLEMAN

1,727,964

## METHOD OF HEAT TREATING PLASTIC AND OTHER MATERIAL

Filed April 13, 1923



Witness:  
R. Burkhardt

Inventor:  
Roy E. Coleman,  
By Wilkinson, Haskay, Byrom & Knobles

## UNITED STATES PATENT OFFICE.

ROY E. COLEMAN, OF CHICAGO, ILLINOIS, ASSIGNOR TO ECONOMY FUSE & MANUFACTURING CO., OF CHICAGO, ILLINOIS, A CORPORATION OF NEW YORK.

## METHOD OF HEAT TREATING PLASTIC AND OTHER MATERIAL.

Application filed April 13, 1923. Serial No. 631,866.

This invention relates to methods of heat treating plastic and other material and refers particularly, although not exclusively, to improvements in heat treating articles containing organic and volatile ingredients and which are heated for the purpose of effecting a curing operation by which certain chemical changes result.

My invention is especially useful in curing 10 molded electrical insulating material composed of such ingredients as asbestos for a base, gilsonite, pitch or other similar material for a binder, oils which under the effect of heat will combine chemically with sulphur 15 or other hardening agent, or will themselves polymerize under heat to give the material hardness, and a volatile oil to give the mass plasticity while molding. The volatile oils may be relatively heavy, such as coil tar oil 20 or paraffin oils which are driven off during the heating or curing operation, or may be relatively light oils, such as naphtha, gasoline, or benzol, which evaporate to a large extent even during the process of mixing and molding 25 the various ingredients.

It has been customary heretofore to cure the molded material of the character described by placing it in a furnace or oven where it is subjected to a relatively high heat 30 from an external source, such as gas burners, while at the same time air is allowed to circulate through the oven to assist in withdrawing the volatilized fumes therefrom.

I have found that by using the process as 35 above described there are many disadvantages. On account of the presence of air at a high temperature, the surfaces of the molded articles become covered with a layer of oxidized oils and other material and prevent 40 the escape of the volatile ingredients in the interior of the article. In order to drive off these volatile ingredients through the oxidized surface excessive heat is required, which causes an overcuring of the surface 45 and results in lack of uniformity throughout the body of the material. Moreover, the extent to which the temperature can be increased is distinctly limited, as with the increase of temperature, the danger of injuring 50 the material by fire also increases.

An object of the present invention is to provide a method of heat treating materials by which the period of time required for complete treatment is materially reduced and a better product is obtained.

A further object is to provide a method of heat treatment which will combine the advantages of uniformity of temperature with perfect control of the atmosphere in which the treatment is carried on.

A further object is to provide a method of heat treatment by which the temperatures required for perfect treatment may be materially reduced.

A further object is to provide a method of heat treating materials containing volatile constituents which will facilitate the removal of said volatile constituents.

A further object is to provide an improved method of heat treatment of materials containing oxidizable constituents which will permit expeditious treatment without danger from oxidation or burning.

A further object is to provide a method of heat treatment according to which the proportions of the various constituents of the treating atmosphere may be readily controlled.

A further object is to provide a method of curing molding material by which curing may be accomplished expeditiously without danger of premature surface curing.

A further object is to provide a method of rapidly curing molded material in which the risk of fire is minimized.

I have discovered that greatly improved results may be obtained in the curing of molded material of the character mentioned by introducing into the heating chamber or oven dry or superheated steam, so that the curing operation is carried out without the presence 85 of air. By providing for a rapid and free circulation of dry steam throughout the heating chamber, the heat within the same is kept evenly distributed, while at the same time oxidation of the surface of the material being 90 cured is prevented. The result of the latter is that the volatile oils have an opportunity to readily escape, and, in fact, their distillation is greatly facilitated by the presence of 95 the steam itself, particularly in the case of 100

heavy oils. In this way the molded articles are much more rapidly cured at a lower temperature than was heretofore possible and a much superior and more uniform product is obtained, while all danger of fire is eliminated.

I have found by actual experience that the time required for curing has been reduced by more than fifty per cent, not only resulting in great economy of operation, but also 10 a much improved product.

My method of treatment is also applicable to a wide variety of uses, among which may be mentioned the drying of certain varnishes, paints, enamels, japans and similar materials 15 applied to the surface of any suitable article. In this case the volatile constituents of the varnish are rapidly driven off in the presence of dry steam. In the case of drying these materials it is advisable to effect a slight 20 oxidation, and this is controlled to exactly the desired extent by admitting a definite proportion of air, which is mixed with the steam to give the desired result.

In the accompanying claims the term "flow- 25 ability conferring agent" is intended to be inclusive of volatile oils for conferring plasticity to insulating material and for conferring fluidity to varnish and the like.

In certain instances it is also possible to 30 use other non-oxidizing gases besides steam, such as carbon dioxide or the like, but in cases in which it is desired to drive off heavy oils I have found that this is effected particularly advantageously by dry or superheated steam.

35 The accompanying drawings illustrate an oven in which my improved method of heat treatment may be used. In the drawings—

Figure 1 is a front elevation, partly in section, illustrating an oven which may be used 40 in carrying out the present invention; and

Figure 2 is a sectional view taken on the line 2—2 of Figure 1.

The oven 1 comprises the outer shell or casing 2 and the inner shell or casing 3. The 45 shells or casings 2 and 3 are sealed together at their uppermost portions, the inner casing 3 preferably being spaced from the outer casing 2 whereby to provide a chamber 4 surrounding said casing 3. The chamber 4 may 50 communicate by means of pipes 5—5 with the outlet main 6. The casing 3 may have the dome-shaped top portion 7 provided with the outlet flue 8.

55 Mounted in the lower portion of the outer casing 2 is the fuel inlet pipe 9, which communicates with the series of burners 10—10, which may be elongated pipes extending from one side of the oven to the other side thereof, as clearly shown in Figure 2. The gas 60 flames from burners 10—10 play upon the under side of the casing 3 to maintain a pre-determined temperature within the casing 3, which temperature should be 100 degrees C. or higher for the purpose of maintaining the 65 steam therein in a dry or superheated condi-

tion. The supply of fuel to the pipe 9 may be controlled by the valve 11. Though the oven has been illustrated with heating means comprising burners, it will be clear that any other preferred heating means may be employed, such, for instance, as electric heaters, heating coils which may contain oil or hot air, or any other type of heater. The type of oven and type of heater constitute no part 70 of the present invention.

75 Communicating with the lower portion of the inner casing 3 is the pipe 12, which may be controlled by means of the valve 13. Said pipe 12, in the practice of the present invention, may conduct steam to the interior of casing 3 for a purpose which will be referred to hereinafter. Also communicating with the lower portion of casing 3 is the pipe 14, which pipe 14 may also have communication with the superheater 15. Steam may be admitted 80 to the casing 3 by way of superheater 15 and pipe 14, the supply of superheated steam being controlled by the valve 16. Pipes 12 and 14 may be extended into the casing 3 to distribute the flow from said pipes 12 and 14 uniformly through said casing 3. A perforated false bottom 17 may be provided near 85 the bottom of the casing 3 to improve the uniformity of the distribution of the steam from the pipes 12 and 14 through the casing 90 3. An inlet pipe 18 may be provided communicating with the bottom part of casing 3 below the false bottom 17 for admitting air, oxygen, or other active gas to said casing 3. Said inlet 18 will be provided with the valve 95 19 for controlling the flow of gas therethrough. The pipes 12 and 14 and the inlet 18 will preferably each be provided with flow meters 20 for the purpose of indicating 100 the flow through their respective pipes. By 105 noting the indications of the flow meters an operator may control to a nicety the relative supplies of inert gas and active gas.

According to the present invention the material is treated in an atmosphere of inert 110 gas, preferably dry steam, said steam being maintained at or above the boiling point of water by any preferred means. In the oven illustrated, the steam entering the casing 3 through pipe 12 is maintained above the boiling point of water by means of the burners 10—10. If preferred, the steam may be superheated before entering the oven, the steam then being introduced through pipe 14 after 115 passing through the superheater 15. In any event, the steam is kept hot and dry. The temperatures of volatilization of the volatile constituents of the material being treated are materially lower in an atmosphere of steam than in an atmosphere of air, and a large proportion of said volatile constituents may be volatilized in an atmosphere of steam 120 at a temperature much lower than is necessary in atmospheric air. The reason why a large 125 proportion of the volatile constituents may be 130

volatilized in an atmosphere of steam at a temperature lower than is necessary in atmospheric air is that in the case of heat treatment in air the flowability conferring agents 5 polymerize excessively, resulting in a rise in temperature due to such polymerization which is very difficult to control. By treating in a flowing inert atmosphere or in an atmosphere containing a regulated amount of air or the 10 like, the polymerization necessary to give hardness is accomplished without undue rise in temperature, any tendency to excessive temperature being minimized due to the flowing inert atmosphere, which acts merely as a 15 vehicle and not as a supply of fuel to unduly promote polymerization. By reason of the lower temperature required, premature surface curing is avoided. Furthermore, by reason of the fact that in an atmosphere of steam 20 there is a minimum, if any, oxidation, a stronger circulation and more even distribution of heat may be provided than is feasible with atmospheric air, and also the volatile constituents of the material being cured 25 may thus be more rapidly carried off. By reason of the fact that premature surface curing is avoided, the liability of warping, cracking and blistering, which are common in air treatment, is minimized.

30 In certain heat treatments of materials, such as the drying of certain varnishes, paints, enamels, japans and similar materials, there is a decided advantage in supplying a limited amount of air to the materials 35 being treated. Difficulty is encountered, however, if the supply of air is merely throttled, due to the fact that a relatively rapid flow of gases is required through the oven to provide the necessary circulation, distribution 40 of heat, and carrying off of volatile products coming from the material being treated. According to the present invention, the relative supplies of dry steam and air, or other active material, are controlled by the valves 13, 16 45 and 19. The dry steam admitted through the steam pipes acts as a carrier for the desired limited amount of air or other active gas, whereby a rapid circulation of gases is maintained through the oven, while any excess of air or other active gas is avoided.

The characteristics of the product resulting from the use of my improved method may be controlled by varying the amount of steam or other gas used at the different stages of 55 the process, or by varying the temperatures used, or by varying both the amount of steam or other gas and the temperature. Furthermore, the chemical composition and the shape and size of the articles being treated will be 60 factors in the determination of the specific procedure followed, this being determinable by simple experimentation in individual cases.

It will be clear that many modifications of 65 the exact method which I have described will

occur to those skilled in the art. It is intended in this patent to cover all such modifications that fall within the scope of the invention as defined by the appended claims.

I claim:

1. The method of treating material having as important constituents thereof a base and a flowability conferring agent, the latter of which includes a volatile oil, which consists in heat treating said material in flowing inert atmosphere maintained in dry condition, said inert atmosphere being maintained at a temperature sufficient for curing said material, the rate of flow being sufficient to hold down the polymerizing effects of said flowability conferring agent to prevent such polymerization from causing an undue rise in temperature.

2. The method of treating material having as important constituents thereof a base and a flowability conferring agent, the latter of which includes a volatile oil, which consists in heat treating said material in an atmosphere of flowing steam maintained in dry condition at a temperature sufficient for curing said material, the rate of flow being sufficient to hold down the polymerizing effects of said flowability conferring agent to prevent such polymerization from causing an undue rise in temperature.

3. The method of treating material having as important constituents thereof a base and a flowability conferring agent, the latter of which includes a volatile oil, which consists in heat treating said material in a flowing inert atmosphere mixed with a predetermined amount of oxygen containing gas, said inert atmosphere and oxygen containing gas being maintained in dry condition at a temperature sufficient for curing said material, the rate of flow being sufficient to hold down the polymerizing effects of said flowability conferring agent to prevent such polymerization from causing an undue rise in temperature.

Signed at Chicago, Illinois, this 10th day of April, 1923.

ROY E. COLEMAN.

115

120

125

130